

## UNITED STATES PATENT OFFICE

2,611,745

## LUBRICATING COMPOSITION

Egbert Mason Kipp, New Kensington, Pa., assignor to Aluminum Company of America, Pittsburgh, Pa., a corporation of Pennsylvania

No Drawing. Application December 17, 1949, Serial No. 133,684. In Canada June 10, 1947

3 Claims. (Cl. 252—49.6)

1

This invention relates to improved lubricants, such as oils, greases or semi-fluid oils, containing as a major lubricating component hydrocarbon oil of natural or synthetic origin. In particular, the invention relates to lubricating compositions of this type having improved extreme pressure characteristics.

Requirements upon lubricants by developments in mechanical design are rigid and drastic. In many instances pressures at bearing surfaces are higher than those which petroleum oils will normally withstand. Illustrative are the conditions encountered in the lubrication of automotive hypoid gears, heavily loaded mill pinion gears, naval turret gears, and the like. In many machines operation is, at least in part, under conditions of thin film lubrication or under similar conditions where film strength, oiliness and anti-wear characteristics of high order are required of the lubricating medium.

The principal object of this invention is the provision of a new composition of matter consisting of a compounded lubricating product possessing extreme pressure characteristics of a high order. Further objects include the provision of a compounded lubricant containing as a major hydrocarbon lubricating component which may be oil or grease of natural or synthetic origin, the lubricant having a superior combination of high film strength, oiliness and anti-wear characteristics.

In accordance with this invention these objects are achieved in substantial part by providing a lubricant, the essential lubricating components of which are a major amount of a hydrocarbon lubricating component which may be oil or grease and a minor amount of a body of boron fluoride and a substance selected from the class consisting of unmodified alcohols containing at least 3 carbon atoms, alcohol-ethers and ethers more specifically described below. The proportion of this body to the hydrocarbon component should be such, however, that the mixture contains at least 0.001 per cent by weight of boron fluoride ( $BF_3$ ) while, on the other hand, more than 3 per cent does not improve the lubricant. Within this range it has been found that the best results are obtained by providing from 0.1 to 1.0 per cent of boron fluoride in the final lubricant mixture. The choice of the particular body to be employed and its boron fluoride content will of course depend on such matters as cost, ease of mixing and the nature of the lubrication problem.

The principal advantages and effectiveness of this new compounded lubricant are maintained

when, in addition to the above mentioned essential components there are likewise present in the lubricating composition other components added to improve some specific characteristic or property thereof, such as viscosity, pour point, oiliness, flow anti-wear characteristics, film strength or the like, the effect of the defined boron fluoride-containing body, when similar, being largely additive. Such diluents or additions may therefore, for the purposes of this invention be regarded as a non-essential portion of the composition, regardless of their specific beneficial or functional effect. The same may be said of substances known as extreme pressure additives, such as substances composed of chlorine, sulphur or lead containing compounds or materials, it being observable that the presence of the defined boron fluoride-containing bodies is effective to increase the extreme pressure characteristics of the compositions even when other extreme pressure additives are present.

The organic  $BF_3$  body, which in accordance with this invention is blended with the hydrocarbon component, may be prepared in various ways but is, for the most part, conveniently prepared by exposing the unmodified alcohol, alcohol-ether or ether to direct contact with gaseous  $BF_3$ . This can be easily accomplished under ordinary atmospheric pressure by bubbling the gaseous  $BF_3$  through the alcohol, alcohol-ether or ether in a liquid state. If the organic material is not liquid at room temperature it should be heated to and maintained at a temperature slightly above its melting point, say 5 or 10° C. Although the rate of flow of the gas is not critical with respect to formation of the  $BF_3$  additive yet the flow should be controlled to avoid undue loss. The rate of acceptance of the  $BF_3$  by the alcohol, alcohol-ether or ether is improved if the liquid is stirred as the gas is introduced. The amount of  $BF_3$  accepted by the alcohol, alcohol-ether or ether is indicated by the increase in weight of the treated mass. The introduction of the gas may therefore be continued until a predetermined increase in weight, short of saturation, has been obtained or the flow of gas may be prolonged until no further increase in weight is observed at which point the alcohol, alcohol-ether or ether is considered to be saturated with  $BF_3$ . Generally, it is most convenient to follow the latter procedure. In both cases, however, the length of time required to reach the end point can be easily determined for the material being treated and thus make it possible to introduce 55 the desired amount of  $BF_3$  without having to test

a charge at intervals during the period of treatment. Although each alcohol, alcohol-ether or ether may have a different saturation point or the desired  $\text{BF}_3$  content may differ for various materials, this does not detract from the value of the  $\text{BF}_3$ -containing body in improving the load bearing quality of a hydrocarbon lubricant.

Other methods of introducing  $\text{BF}_3$  can be employed, of course. For example, the alcohol, alcohol-ether or ether may be exposed to the gas at higher temperatures and pressures and thus shorten the time required to introduce the desired amount of  $\text{BF}_3$ . Naturally, the temperature and pressure should be such that the alcohol, alcohol-ether or ether is not decomposed to any substantial degree. Another method of contacting the organic material with  $\text{BF}_3$  is to add compounds to it which can be decomposed with the release of  $\text{BF}_3$ . Such compounds as  $\text{NH}_3\text{BF}_4$ ,  $\text{BF}_3\cdot\text{NH}_3$ , the heavy metal fluoborates or even other organic materials previously treated with  $\text{BF}_3$  may be employed. To effect decomposition it is usually necessary to heat the mixture of alcohol, alcohol-ether or ether and the  $\text{BF}_3$ -containing substance. Further, it may be desirable to remove any residues resulting from the decomposition.

The amount of  $\text{BF}_3$  that can be introduced into different alcohols, alcohol-ethers or ethers will vary, as mentioned above, however, from 10 to 20 per cent by weight is preferred where the saturation point permits it. In any case, the alcohols, alcohol-ethers or ethers should be treated with sufficient fluoride to provide the desired  $\text{BF}_3$  content in the lubricating composition as only a minor proportion of the additive is employed.

The resultant product may, in some instances, be an actual compound, there being some evidence to indicate that such is its nature, or it may be an additive or coordinate compound or even a solution or dispersion. I prefer, however, to term the product a body or composition consisting essentially of a substance selected from the class consisting of unmodified alcohols containing at least 3 carbon atoms, alcohol-ethers and ethers and  $\text{BF}_3$  and, therefore, not to characterize the state of association of the fluoride and the organic substance. In any event, the unmodified alcohols containing at least 3 carbon atoms, alcohol-ethers and ethers act as acceptors of  $\text{BF}_3$  to produce a body or substance having positive advantages as an additive in lubricating compositions.

The following list of alcohols, alcohol-ethers and ethers is illustrative of the class which when treated with  $\text{BF}_3$  produce the bodies just described: straight chain normal alkyl monohydric alcohols such as propyl through octadecanol as well as higher molecular weight alcohols of the type represented by tetracosanol and triacontanol; alkyl, aromatic, and cyclic (and polyhydroxy derivatives thereof) ethers of mono- and polyhydric alkyl, aromatic and cyclic alcohols such as ethylene glycol monomethyl ether, ethylene glycol diethyl ether, ethylene glycol mono octadecyl ether, ethylene glycol ethylbutyl ether, ethylene glycol monophenyl ether, ethylene glycol monobenzyl ether, diethylene glycol diethyl ether, tetraethylene glycol dimethyl ether, propylene glycol methyl ether, propylene glycol 4-biphenyl ether, tripropylene glycol n-butyl ether, polypropylene glycol methyl ether (mol. wt. 496 to 3000), dodecyl 2,3-dihydroxypropyl ether, 1,3-dihydroxypropyl-2 hexadecyl ether, phenyl decyl ether, p-tolyl dodecyl ether, naphthyl undecyl ether, hydroxycyclohexyl octadecyl ether and

resorcinol mono pentadecyl ether; alkyl, aromatic and cyclic ethers of pentaerythritol, mannitol, sorbitol and allied polyhydroxy compounds; normal alkyl and branched chain alkyl ethers, simple, mixed, symmetrical and unsymmetrical butyl through octadecyl.

The introduction of the  $\text{BF}_3$  into the unmodified alcohols, alcohol-ethers and ethers may change the color thereof, often making it darker. Also, the liquid alcohol, alcohol-ether or ether may become thicker as the introduction of  $\text{BF}_3$  proceeds and the melting point of the end product may be higher than that of the original alcohol, alcohol-ether or ether. Such changes do not affect the advantages gained from the presence of the  $\text{BF}_3$ -containing bodies in a hydrocarbon lubricant, certainly the results of the invention do not depend upon or are responsive to any peculiar chemical or physical qualities of the  $\text{BF}_3$ -containing additive, rather they depend upon the admixture of the additive with the hydrocarbon lubricant.

The action of these organic  $\text{BF}_3$  bodies in a hydrocarbon lubricant is positive and specific to increase the load bearing capacity of the lubricant and, in many instances, to definitely improve its anti-wear characteristics. The amount of these organic  $\text{BF}_3$  bodies necessarily present to produce these specific effects is very small. The amounts used, should in any case, as mentioned above, provide at least 0.001 per cent by weight of  $\text{BF}_3$  in the final mixture. The amount of any given  $\text{BF}_3$ -containing body desirably present to produce optimum effects in any particular hydrocarbon lubricant can be readily determined by simple trial, the optimum usually being found within the range of 0.5 to 5 per cent by weight of the alcohol, alcohol-ether or ether  $\text{BF}_3$  body. Amounts below about 0.01 per cent by weight often do not produce sufficient effect to be usually characterized as commercial, but the effect produced is such as to be useful under exceptional conditions. One may use a relatively small amount of an additive containing a substantial quantity of  $\text{BF}_3$  or a larger amount of the same or another additive which contains a smaller proportion of  $\text{BF}_3$  to introduce a given quantity of  $\text{BF}_3$  into the hydrocarbon component. In any event, the organic  $\text{BF}_3$ -additive forms a minor amount or proportion of the lubricating composition.

The load bearing qualities of a lubricant may be relatively determined by various methods. The method used to obtain the comparative data hereinafter set forth is practiced on a Falex machine and consists in submitting small quantities of the lubricant to the action of a rotating steel journal rotated in contact with two V-shaped bearing blocks. During testing measurable pressure was applied to the rotating journal by use of an automatic loading device. The two bearing blocks and the journal were submerged in the lubricant sample throughout the tests. In each test load was applied and allowed to reach 500 pounds; at this load the journal was then run for 5 minutes; thereafter the load was gradually increased until lubrication failure occurred. The load at the time of failure is designated as the failure load. In general, the failure loads are reproducible within 150 pounds at lower pressure and 300 pounds at higher pressure; the results are not absolute but are comparative with a standard run under the same conditions. In the tests by which the results set forth in the following table were secured, the hydrocarbon oil was in all cases

the same, being a straight mineral oil. In all cases 1 per cent by weight of additive was present in the oil. The additive had been prepared by passing  $\text{BF}_3$  through the alcohol, alcohol-ether or ether until the weight of the body became substantially constant, that is, the organic material became saturated with the  $\text{BF}_3$ , as has been described hereinabove. Each comparative test was run on two samples, one sample being the oil containing 1 per cent by weight of an alcohol, alcohol-ether or ether, the other sample being the oil containing the same weight of a  $\text{BF}_3$ -containing body. In the first column of the table the nature of the additive is set forth, in the second column is listed the  $\text{BF}_3$  content of the treated material, in the third column is the  $\text{BF}_3$  content of the lubricant, in the fourth column the failure load in pounds is given and in the fifth column is shown the percentage increase in failure load caused by the presence of the  $\text{BF}_3$ -containing body.

consisting essentially of a substance selected from the class consisting of unmodified alcohols containing at least three carbon atoms, alcohol-ethers and ethers and  $\text{BF}_3$ , said body being prepared by exposing said substances to direct contact with a substance selected from the class consisting of gaseous  $\text{BF}_3$  and decomposable compounds yielding gaseous  $\text{BF}_3$  and being present in such amount that the lubricating composition contains from 0.001 to 3 per cent by weight of  $\text{BF}_3$ , said lubricating composition possessing extreme pressure characteristics superior to those exhibited by a similar composition in which the minor proportion aforesaid consists of said substance selected from the class consisting of unmodified alcohols, alcohol-ether and ethers.

2. A lubricating composition comprising a major proportion of a hydrocarbon lubricating oil blended with a minor proportion of a body consisting essentially of cetyl alcohol and  $\text{BF}_3$ , said body being prepared by exposing cetyl alco-

| Additive                            | Percent $\text{BF}_3$ in Additive | Percent $\text{BF}_3$ in Lubricant | Failure Load in Pounds | Percent-<br>age Increase |
|-------------------------------------|-----------------------------------|------------------------------------|------------------------|--------------------------|
| Octyl alcohol                       |                                   |                                    | 500                    |                          |
| Octyl alcohol + $\text{BF}_3$       | 38.                               | .38                                | 14,000                 | 1700                     |
| Tetradecanol                        |                                   |                                    | 880                    |                          |
| Tetradecanol + $\text{BF}_3$        | 24.                               | .24                                | 3,950                  | 348                      |
| Cetyl alcohol                       |                                   |                                    | 1,150                  |                          |
| Cetyl alcohol + $\text{BF}_3$       | 19.8                              | .2                                 | 3,500                  | 204                      |
| Polyethylene glycol (mol. wt. 200)  |                                   |                                    | 880                    |                          |
| Polyethylene glycol + $\text{BF}_3$ | 48.                               | .48                                | 1,650                  | 87                       |
| Phenyl cellosolve                   |                                   |                                    | 750                    |                          |
| Phenyl cellosolve + $\text{BF}_3$   | 39.                               | .39                                | 2,100                  | 180                      |
| Methyl cellosolve                   |                                   |                                    | 750                    |                          |
| Methyl cellosolve + $\text{BF}_3$   | 64.                               | .64                                | 1,950                  | 160                      |
| Diethyl cellosolve                  |                                   |                                    | 750                    |                          |
| Diethyl cellosolve + $\text{BF}_3$  | 54.5                              | .55                                | 1,450                  | 90                       |
| Diethyl carbitol                    |                                   |                                    | 800                    |                          |
| Diethyl carbitol + $\text{BF}_3$    | 50.                               | .5                                 | 2,110                  | 163                      |
| N-Hexyl ether                       |                                   |                                    | 800                    |                          |
| N-Hexyl ether + $\text{BF}_3$       | 28.3                              | .28                                | 2,350                  | 193                      |

<sup>1</sup> Greater than.

"Cellosolve" used in the above tabulation designated the glycol monethyl ether sometimes designated as 2-ethoxy-ethanol while "carbitol" designates diethylene glycol monoethyl ether.

The machine on which the tests were run had a capacity of 4500 pounds. Where this capacity was approximated or exceeded the failure load is indicated above as being greater than 4000 pounds. These tabulated results are indicative of the improvement obtained by the practice of this invention. In general, torque and temperature values obtained during these tests indicated that the organic  $\text{BF}_3$  body improved friction qualities and observations simultaneously made indicated increases in anti-wear characteristics.

In compounding lubricant compositions of the type herein described and claimed the organic  $\text{BF}_3$  additive may merely be mixed with the hydrocarbon lubricants, the properties of which are to be improved. Where the additive is insoluble in the lubricant or it is desired to incorporate therein amounts in excess of solubility, emulsions or dispersions may be prepared according to known principles.

This application is a continuation-in-part of my prior application Serial No. 714,910 filed December 7, 1946, and entitled Lubrication Composition, now abandoned.

Having thus described my invention and the known advantages thereof, I claim:

1. A lubricating composition comprising a major proportion of a hydrocarbon lubricating oil blended with a minor proportion of a body

50 hol to direct contact with a substance selected from the class consisting of gaseous  $\text{BF}_3$  and decomposable compounds yielding gaseous  $\text{BF}_3$  and being present in such amount that the lubricating composition contains from 0.001 to 3 per cent by weight of  $\text{BF}_3$ , said lubricating composition possessing extreme pressure characteristics superior to those exhibited by a similar composition in which the minor proportion aforesaid consists of cetyl alcohol.

60 3. A lubricating composition comprising a major proportion of a hydrocarbon lubricating oil blended with a minor proportion of a body consisting essentially of octyl alcohol and  $\text{BF}_3$ , said body being prepared by exposing octyl alcohol to direct contact with a substance selected from the class consisting of gaseous  $\text{BF}_3$  and decomposable compounds yielding gaseous  $\text{BF}_3$  and being present in such amount that the lubricating composition contains from 0.001 to 3 per cent by weight of  $\text{BF}_3$ , said lubricating composition possessing extreme pressure characteristics superior to those exhibited by a similar composition in which the minor proportion aforesaid consists of octyl alcohol.

65 EGBERT MASON KIPP.

## REFERENCES CITED

The following references are of record in the file of this patent:

## UNITED STATES PATENTS

| Number    | Name      | Date          |
|-----------|-----------|---------------|
| 2,053,474 | Graves    | Sept. 8, 1936 |
| 2,160,917 | Shoemaker | June 6, 1939  |
| 2,266,060 | Miller    | Dec. 16, 1941 |

## FOREIGN PATENTS

| Number  | Country       | Date         |
|---------|---------------|--------------|
| 645,202 | Great Britain | Jan. 9, 1948 |
| 645,425 | Great Britain | Jan. 9, 1948 |

## OTHER REFERENCES

Boron Trifluoride and its Derivatives—Booth et al., John Wiley and Sons—1949, pp. 61-64 and 68-71.